



US007521870B2

(12) **United States Patent**  
**Watanabe et al.**

(10) **Patent No.:** **US 7,521,870 B2**  
(b5) **Date of Patent:** **Apr. 21, 2009**

(54) **LUMINOUS CONTAINERS AND THOSE FOR HIGH PRESSURE DISCHARGE LAMPS**

(75) Inventors: **Keiichiro Watanabe**, Kasugai (JP); **Takashi Ohta**, Kasugai (JP); **Naoki Masui**, Kounan (JP)

(73) Assignees: **NGK Insulators, Ltd.**, Nagoya (JP); **NGK Optoceramics Co., Ltd.**, Komaki (JP)

(\*) Notice: Subject to any disclaimer, the term of this patent is extended or adjusted under 35 U.S.C. 154(b) by 687 days.

(21) Appl. No.: **11/144,369**

(22) Filed: **Jun. 3, 2005**

(65) **Prior Publication Data**

US 2006/0022596 A1 Feb. 2, 2006

**Related U.S. Application Data**

(60) Provisional application No. 60/604,319, filed on Aug. 25, 2004.

(30) **Foreign Application Priority Data**

Jun. 8, 2004 (JP) ..... P2004-169497  
Aug. 11, 2004 (JP) ..... P2004-234670

(51) **Int. Cl.**  
**H01J 1/88** (2006.01)

(52) **U.S. Cl.** ..... **313/623; 313/285**

(58) **Field of Classification Search** ..... **313/623-625, 313/283-290, 253, 252, 244, 243**

See application file for complete search history.

(56) **References Cited**

U.S. PATENT DOCUMENTS

3,531,853 A 10/1970 Klomp  
3,564,328 A 2/1971 Bagley et al.

|                  |         |                             |
|------------------|---------|-----------------------------|
| 3,848,151 A      | 11/1974 | McVey                       |
| 4,011,480 A      | 3/1977  | Jacobs et al.               |
| 4,376,905 A      | 3/1983  | Kerekes                     |
| 4,459,509 A      | 7/1984  | Csapody et al.              |
| 4,746,582 A      | 5/1988  | Tsuno                       |
| 4,803,403 A      | 2/1989  | Makar, Jr. et al.           |
| 5,404,077 A      | 4/1995  | Eichelbrönnér et al.        |
| 6,027,389 A      | 2/2000  | Miyazawa et al.             |
| 6,262,533 B1     | 7/2001  | Niimi                       |
| 2004/0086298 A1  | 5/2004  | Ojima et al.                |
| 2005/0236960 A1* | 10/2005 | Kupper et al. ..... 313/489 |

FOREIGN PATENT DOCUMENTS

GB 1 435 244 5/1976

(Continued)

OTHER PUBLICATIONS

U.S. Appl. No. 11/391,945, filed Mar. 29, 2006, Watanabe et al.

Primary Examiner—Nimeshkumar D. Patel

Assistant Examiner—Christopher M Raabe

(74) Attorney, Agent, or Firm—Burr & Brown

(57) **ABSTRACT**

A luminous container has an electrode supporting member composed of a pipe-shaped metal piece. The electrode supporting member **8** has a clamped portion pressed and clamped with and non-clamped portions not clamped with a brittle material. The stress generated along a contact interface of the clamped portion and the brittle material is relaxed with the deformation of the electrode supporting member.

**32 Claims, 34 Drawing Sheets**



## FOREIGN PATENT DOCUMENTS

|    |           |         |    |             |         |
|----|-----------|---------|----|-------------|---------|
| JP | 41-7815   | 4/1966  | JP | 63-159264   | 7/1988  |
| JP | 45-10627  | 5/1970  | JP | 63-259958   | 10/1988 |
| JP | 50-45482  | 4/1975  | JP | 05 205701   | 8/1993  |
| JP | 50-78175  | 6/1975  | JP | 06-296107   | 10/1994 |
| JP | 51-72187  | 6/1976  | JP | 07-33294    | 4/1995  |
| JP | 52-080675 | 7/1977  | JP | 10-125230   | 5/1998  |
| JP | 56-128561 | 10/1981 | JP | 11-149902   | 6/1999  |
| JP | 57-046562 | 3/1982  | JP | 11-265686   | 9/1999  |
| JP | 57-145261 | 9/1982  | JP | 2004-134219 | 4/2004  |
| JP | 60-59352  | 4/1985  | JP | 2004-149640 | 5/2004  |
| JP | 62-182174 | 8/1987  | JP | 2004-163911 | 6/2004  |

\* cited by examiner



Fig. 1

Fig. 2



3  
正



Fig. 4



۵۰



Fig. 6



Fig. 7



Fig. 8





၁၁၁

Fig. 10



Fig. 11



Fig. 12



Fig. 13





Fig. 15



Fig. 16



Fig. 17





Fig. 19



Fig. 20



Fig 21



Fig. 22



Fig. 23



Fig. 24



Fig. 25



Fig. 26



Fig. 27



Fig. 28



Fig. 29



Fig. 30



Fig. 31





Fig. 33





## 1

## LUMINOUS CONTAINERS AND THOSE FOR HIGH PRESSURE DISCHARGE LAMPS

## CROSS-REFERENCE TO RELATED APPLICATIONS

This application claims the benefit of Japanese patent application 2004-169497, filed on Jun. 8, 2004, Japanese patent application 2004-234670, filed on Aug. 11, 2004, and U.S. patent application 60/604,319, filed on Aug. 25, 2004, the entireties of which are incorporated by reference.

## FIELD OF THE INVENTION

The present invention relates to a luminous container suitable for use in a high pressure discharge lamp or the like.

## BACKGROUND OF THE INVENTION

According to a luminous container for a high pressure discharge lamp described in Japanese patent publication 10-125230A, a molded body for a main body of a tube and a ring-shaped sealing member for the end portion are separately produced, and the two kinds of the molded bodies are assembled to produce an assembly. The assembly is then sintered to produce a container for sealing metal halide. In the process, the sintering shrinkages of both molded bodies are designed so that the outer diameter of the sintered body of the molded body for the sealing member for the end portion is larger than the inner diameter of the molded body for the main body for the tube, if each of the molded bodies would have been sintered alone. During the sintering, a clamping force is applied from the main body of the tube toward the sealing member for the end portion so that both sintered bodies are bonded in good manner to preserve excellent air-tightness.

For example, according to a luminous container for a high pressure discharge lamp listed in Japanese patent publication 10-125230A, a ring-shaped sealing member is pressed onto the end portion of the luminous vessel and an electrode member is inserted into a through hole of the sealing member. The sealing member is made of a cermet and the luminous vessel is made of a ceramic material such as alumina. The molded body for the sealing member is fixed in the opening in the end portion of the molded body for luminous vessel, and the molded bodies are then sintered to shrink them. In this process, it is designed that the shrinkage percentage of the luminous vessel is made larger than that of the sealing member. It is thus possible to generate compressive force from the luminous tube toward the sealing member to fix the sealing member in air-tight manner. A metal electrode member is inserted into the opening of the sealing member to seal the sealing member and electrode member in air-tight manner.

## SUMMARY OF THE INVENTION

According to the method of sealing the end portion as described in Japanese patent publication 10-125230A, metal welding cannot be applied for sealing the sealing and electrode members, so that glass or metal oxide cement has been used for the sealing. Glass or metal oxide cement is relatively weak against a corrosion substance such as metal halide gas at high temperature and susceptible to corrosion. Further, these materials are susceptible to fracture by many times of thermal cycles of high and low temperatures and thus have a limitation in the reliability.

An object of the present invention is to provide a luminous container for sealing a luminous substance in a brittle mate-

## 2

rial in air-tight manner and alleviating the necessity of the direct contact of the sealing material with a corrosive substance.

5 A first aspect of the present invention provides a luminous container comprising an electrode supporting member comprising a plate-shaped metal piece preferably having a shape of a seamless cylinder, said electrode supporting member comprising a clamped portion pressed and clamped with and a non-clamped portion not clamped with a brittle material, wherein a stress generated along an interface of the clamped portion and brittle material is relaxed by the deformation of the electrode supporting member.

10 Further, a first aspect of the present invention provides a luminous container for a high pressure discharge lamp comprising the luminous vessel, an electrode and a current through conductor both supported by the electrode supporting member.

15 A second aspect of the present invention further provides a luminous container comprising an outer supporting body comprising a tube-shaped portion of a brittle material, an inner supporting body provided inside of said outer supporting body and made of a brittle material, and a plate-shaped metal piece provided between said outer supporting body and said inner supporting body. The outer supporting body and the plate-shaped metal piece directly contact each other, the plate-shaped metal piece and the inner supporting body directly contact each other and the outer supporting body and the inner supporting body directly contact each other.

20 A second aspect of the present invention further provides a luminous container comprising an inner supporting body comprising a tube-shaped portion made of a brittle material, an outer supporting body provided outside of said inner supporting body and made of a brittle material, and a plate-shaped metal piece provided between said inner and outer supporting bodies. The inner supporting body and the plate-shaped metal piece directly contact each other, the plate-shaped metal piece and the outer supporting body directly contact each other and the inner supporting body and the outer supporting body directly contact each other.

25 The aspect of the present invention further provides a luminous container for a high pressure discharge lamp having the luminous container, a current through conductor and an electrode both supported by the electrode supporting member.

30 Accordingly, the luminous container of the present invention, an electrode supporting member composed of a plate-shaped metal piece is pressed with a brittle material so as to seal luminous substance in air-tight manner. Such structure does not require frit glass and cement materials directly contacting the luminous substance essential for prior structures, so that the resulting luminous container is expected to have improved corrosion resistance against the luminous substance.

35 Further, according to the luminous container of the third aspect, it is provided an outer supporting body comprising a ceramics or cermet, an inner supporting body comprising a ceramic or a cermet, and a clamped portion of a plate-shaped metal piece sandwiched by the outer and inner supporting bodies, so that the clamped portion of the plate-shaped metal piece is pressed by the outer and inner supporting bodies. It is thus possible to pressure bond the metal piece with cermet or ceramics to provide a novel structure, preferably for air-tight sealing. According to prior arts, it is known as a pinch seal, in 40 which a metal foil is inserted into an opening at the end of a glass container and the glass is soften and deformed to provide air-tight sealing using the metal foil. It has not been

known to provide air-tight sealing using brittle materials such as ceramics or cermet which is resistive to softening and deformation.

The brittle material for pressing the electrode supporting member or forming the main body of the luminous container is not particularly limited according to the present invention, and includes glass, ceramics, single crystal and cermet.

Such glass includes quartz glass, aluminum silicate glass, borosilicate glass, silica-alumina-lithium series crystallized glass etc.

The ceramics includes, for example, ceramics having corrosion resistance against a halogen series corrosive gas, and may preferably be alumina, yttria, yttrium-aluminum garnet, aluminum nitride, silicon nitride or silicon carbide. Single crystals of any of the materials selected from the above may be used.

The cermet may be composite materials of a ceramics such as alumina, yttria, yttrium-aluminum garnet and aluminum nitride and a metal such as molybdenum, tungsten, hafnium and rhenium.

The single crystal includes those being optically transparent in visual ray band, such as diamond (single crystal of carbon) or sapphire (Al<sub>2</sub>O<sub>3</sub> single crystal).

According to the present invention, the electrode supporting member made of the plate-shaped metal piece and preferably having a shape of a seamless cylinder has a clamped portion pressed and clamped with a brittle material and a non-clamped portion not pressed and not clamped with the brittle material. The brittle material clamping the plate-shaped metal piece may be a luminous vessel or a plug member fixed in the inside of an end portion of a luminous vessel. Alternatively, the brittle material may be a clamping member fixed to the outside of the end portion of the luminous vessel. Further, outer and inner supporting bodies each made of a brittle material separate from the luminous vessel may be prepared to clamp the plate-shaped metal piece between the outer and inner supporting bodies, so that the outer and inner supporting bodies are bonded to the luminous vessel.

According to the present invention, the plate-shaped metal material may preferably be pressed and clamped at both sides in the direction of thickness with brittle materials having thermal expansion coefficients being substantially equivalent or same with each other. It is thus possible to avoid the generation of stress between the opposing brittle material portions. Stress generated in the metal member provides substantially equivalent distribution with respect to the central plane passing through the center of the metal member in the direction of thickness. Further, the metal member has a thickness considerably smaller than that of the brittle material, so that the stress generated in the metal member is relaxed by the plastic deformation of the metal. It is thus possible to avoid the possibility of critical damages such as bending and crack formation of the metal member or considerable deformation, after the press clamping while under temperature change conditions.

According to the present invention, the stress generated along the contact interface between the clamped portion and the brittle material is relaxed due to the deformation of the plate-shaped metal piece.

The stress along the contact interface of the clamped portion and brittle material is generated, for example, due to the following mechanism. The thermal expansion coefficient of the metal material is represented by " $\alpha_1$ ", the Young's modulus of the metal is represented by " $E_1$ ", the thermal expansion coefficient of the brittle material is represented by " $\alpha_2$ " and the Young's modulus of the brittle material is represented by " $E_2$ ". It is now provided that the metal material is embedded

in the brittle material, and the brittle material is then sintered at a sintering temperature " $T_1$ " and cooled to room temperature so that the metal material is pressed and clamped with the brittle material. In this case, it is provided that both materials would not be deformed and would not slide along the interface, the stress " $\sigma_1$ " generated in the metal is represented by the following formula.

$$\sigma_1 \propto E_1 \times (T_1 - \text{room temperature}) \times (\alpha_1 - \alpha_2) \quad (1)$$

10 The stress " $\sigma_2$ " generated in the brittle material is similarly represented by the formula.

$$\sigma_2 \propto E_2 \times (T_1 - \text{room temperature}) \times (\alpha_2 - \alpha_1) \quad (2)$$

The combination of molybdenum and alumina is taken for the example, the thermal expansion coefficient and Young's modulus of molybdenum are about 5 ppm/ $^{\circ}$ C. and about 330 GPa, respectively. The thermal expansion coefficient and Young's modulus of alumina are about 8 ppm/ $^{\circ}$ C. and about 360 GPa, respectively. For example, when alumina is sintered at 1500 $^{\circ}$ C. and then cooled to room temperature, a compressive stress of about 1500 MPa is generated in molybdenum, provided that there is not plastic deformation of molybdenum. Similarly, a tensile stress of about 1600 MPa is generated in alumina.

25 Both of the stress values are beyond the strengths of the corresponding materials, so that such composite structure cannot be produced because of the fracture along the interface of the brittle material and metal.

30 However, a stress generated in the metal beyond the yield strength of the metal results in the plastic deformation. The magnitude of the deformation until the fracture is represented by the elongation. Such elongation generally takes a considerably large value of several percent to several tens percent.

35 According to the present invention, the thickness of the metal material is made relatively smaller than that of the ceramic material, so as to generate a stress larger than the yield strength of the metal to cause the plastic deformation, so that the overall stress generated due to the difference of the thermal expansion coefficients is relaxed.

40 For example, it is provided that the metal member is made of a thin plate of molybdenum having a thickness of 100 micrometer, and the ceramic block is made of alumina having a thickness of 10 mm, the strain in the molybdenum plate required for deforming the molybdenum plate and for relaxing the stress is represented by the following formula (3).

$$\epsilon = (T_1 - \text{room temperature}) \times (\alpha_1 - \alpha_2) \approx 0.5\% \quad (3)$$

45 The amount of deformation in the direction of the thickness is represented by the formula.

$$\Delta t = \epsilon \times t \approx 0.5 \text{ micrometer} \quad (4)$$

50 It is thus possible to relax the overall stress by a considerably small amount of deformation.

55 The combination of platinum and alumina is taken for example, the thermal expansion coefficient and Young's modulus of platinum are about 9 ppm/ $^{\circ}$ C. and about 170 GPa, respectively, and the thermal expansion coefficient and Young's modulus of alumina are about 8 ppm/ $^{\circ}$ C. and about 360 GPa, respectively. For example, when alumina is sintered at 1500 $^{\circ}$ C. and then cooled to room temperature, a tensile stress of about 250 MPa is generated in platinum member provided that no plastic deformation is generated in platinum. Similarly, a compressive stress of about 530 MPa is to be generated in the alumina member.

60 Also in this case, when the platinum member is made of a thin plate having a thickness of 100 mm and the alumina member is made of a block having a thickness of 10 mm, the

strain in the platinum member required for deforming the platinum thin plate and for relaxing it is represented by the above formula (3) and about 0.1 percent in this case. Although a tensile stress is generated in the platinum member in the direction of the pressing and clamping, only 0.1 percent of deformation in the direction of the depth of the platinum plate can relax the tensile stress. The amount of deformation is only 10  $\mu\text{m}$ , provided that the depth of the pressing and clamping is 10 mm.

As described above, the stress is generated mainly due to the difference of thermal expansion coefficients of the brittle and metal materials in the composite structure of the materials and thus reflects a strain of about 1 percent or lower. On the other hand, the yield strength of the metal material is lower than the tensile strength and the elongation required for the fracture is several percent to several tens percent. The thickness of the metal material is made relatively smaller than that of the brittle material so as to generate a stress larger than the yield strength of the metal to cause the plastic deformation for relaxing the difference of the thermal expansion coefficients. Even in this case, the amount of deformation is in a range of the elongation so that the fracture of the metal material is avoided. Further, the metal material is deformed to relax the stress generated in the brittle material to provide a composite structure of the brittle material and metal. When the materials are integrated utilizing sintering shrinkage requiring thermal process at a high temperature, the relaxing of the stress can be performed also due to deformation of the metal material such as high temperature creep.

According to a preferred embodiment, the difference of the thermal expansion coefficients of the brittle materials on the both side of the plate-shaped metal piece may preferably be 2 ppm or lower and more preferably be 1 ppm or lower. Most preferably, the thermal expansion coefficients are the same. The thermal expansion coefficients of the both brittle materials may be thus adjusted to further improve the stability and reliability of the inventive structure of brittle material and metal against thermal cycles.

According to a preferred embodiment, brittle materials on the both sides for pressing and clamping the clamped portion of the plate-shaped metal piece is composed of sintered bodies having different sintering shrinkages, so that the plate-shaped metal piece is pressure bonded with the difference of shrinkage during the sintering process. A preferred value of the difference of shrinkages will be described below.

Alternatively, according to a preferred embodiment, brittle materials on the inner side for pressing the material of the clamped portion of the plate-shaped metal piece may be selected from those not subjected to sintering shrinkage such as a sintered body, a single crystal and glass, and the outer brittle material may be composed of a molded body subjected to sintering shrinkage.

According to a preferred embodiment, the thickness of the plate-shaped metal piece may preferably be 1000  $\mu\text{m}$  or smaller, and more preferably be 200  $\mu\text{m}$  or smaller. The thickness of the plate-shaped metal piece may be made smaller as described above, to cause the deformation of the metal piece. It is thus possible to reduce the stress generated between the metal piece and brittle material and to further improve the air-tightness of the structure. If the plate-shaped metal piece is too thin, however, the strength as the structural body tends to be insufficient. On the viewpoint, the thickness of the metal piece may preferably be 20  $\mu\text{m}$  or larger, and more preferably be 50  $\mu\text{m}$  or larger.

According to a preferred embodiment, the outer brittle material pressing and clamping the clamped portion of the plate-shaped metal piece has a thickness of 0.1 mm or larger.

It is thus possible to sufficiently increase the pressure from the brittle material onto the plate-shaped metal piece radially, so as to further improve the air-tightness of the luminous container. On the viewpoint, the thickness of the outer brittle material may preferably be 0.5 mm or larger.

The material and shape of the plate-shaped metal piece is not particularly limited. The material of the metal piece may preferably be a metal having a high melting point. Such metal having a high melting point includes one or more metal(s) selecting from the group consisting of molybdenum, tungsten, rhenium, hafnium, niobium and tantalum, or the alloy containing the metal(s). Further, metal parts other than the plate-shaped metal piece such as the cylindrical portion, ring-shaped portion and capillary portion may be made of the above metal(s) listed for the plate-shaped metal piece.

#### BRIEF DESCRIPTION OF THE DRAWINGS

FIG. 1 is a cross sectional view schematically showing a cylindrical type luminous container of a prior art.

FIG. 2 is a cross sectional view schematically showing a cylindrical type luminous container 1A.

FIG. 3 (a) is a cross sectional view schematically showing an assembly for producing the luminous container 1A, and FIG. 3 (b) is a cross sectional view showing a luminous container obtained by sintering the assembly of FIG. 3 (a).

FIG. 4 is a cross sectional view schematically showing an assembly 1B for a cylindrical type luminous container 1B.

FIG. 5 is a cross sectional view schematically showing a cylindrical type luminous container 1C.

FIG. 6 is a cross sectional view schematically showing a cylindrical type luminous container 1D.

FIG. 7 is a cross sectional view schematically showing a cylindrical type luminous container 1E.

FIG. 8 is a cross sectional view schematically showing a cylindrical type luminous container 1F.

FIG. 9 is a cross sectional view schematically showing a cylindrical type luminous container 1G.

FIG. 10 is a cross sectional view schematically showing an elliptical type luminous container of a prior art.

FIG. 11 is a cross sectional view schematically showing a luminous container 11A of elliptical type (one-body type).

FIG. 12 is a cross sectional view schematically showing a luminous container 11B of elliptical type.

FIG. 13 is a cross sectional view schematically showing a luminous container 11C of elliptical type.

FIG. 14 is a cross sectional view schematically showing a luminous container 11D of elliptical type.

FIG. 15 is a cross sectional view schematically showing a luminous container 11E of elliptical type.

FIG. 16 is a cross sectional view schematically showing an elliptical type luminous container of a prior art.

FIG. 17 is a cross sectional view schematically showing a luminous container 21A of elliptical type (two-body type).

FIG. 18 is a cross sectional view schematically showing a luminous container 21B of elliptical type.

FIG. 19 is a cross sectional view schematically showing a luminous container 21C of elliptical type.

FIG. 20 is a cross sectional view schematically showing a luminous container 21D of elliptical type.

FIG. 21 is a cross sectional view schematically showing a luminous container 21E of elliptical type.

FIG. 22 is a cross sectional view schematically showing an elliptical type luminous container 32 of a prior art.

FIG. 23 is a cross sectional view schematically showing an assembly 31A for a luminous container of elliptical type (one-body type).

FIG. 24 is a cross sectional view schematically showing a luminous container 31B of elliptical type.

FIG. 25 is a cross sectional view schematically showing a luminous container 31C of elliptical type.

FIG. 26 is a cross sectional view schematically showing a luminous container 31D of elliptical type.

FIG. 27 is a cross sectional view schematically showing a luminous container 31E of elliptical type.

FIG. 28 is a cross sectional view schematically showing a luminous container 31F of elliptical type.

FIG. 29 is a cross sectional view schematically showing a luminous container 31G of elliptical type.

FIG. 30 is a cross sectional view schematically showing an HPS type luminous container 42 of a prior art.

FIG. 31 is a cross sectional view schematically showing a luminous container 41A of HPS type.

FIG. 32 is a cross sectional view schematically showing a luminous container 41B of HPS type.

FIG. 33 is a cross sectional view schematically showing an assembly of a luminous container 41C of HPS type.

FIG. 34 is a cross sectional view schematically showing a luminous container 41D of HPS type.

#### DETAILED DESCRIPTION OF THE INVENTION

The present invention will be described concerning the examples, referring to the attached drawings below.

FIG. 1 is a cross sectional view schematically showing a luminous container of a prior art, and FIGS. 2 to 8 are cross sectional views schematically showing luminous containers each using a luminous vessel of so called cylindrical type.

As shown in FIG. 1, an alumina supporting tube 4 is fixed onto the inner wall surface 2a of a luminous vessel 2 having a shape of a straight tube at both ends through a sealing member 3 made of alumina. The supporting tube 4 and a current through conductor 5 are sealed with a sealing material 6 composed of glass frit or the like. According to the structure, luminous substance at high temperature filled in an inner space 7 of a luminous vessel 2 contacts the sealing material 6, so that the corrosion of the sealing member 6 tends to result in a problem in the structure.

Further, although niobium may preferably be applied as the material of the current through conductor 5 having a thermal expansion coefficient near that of a ceramic (alumina), niobium is susceptible to the corrosion by a luminous substance and thus problematic. Therefore, the current through conductor and electrode may be made of three kinds of materials such as niobium-molybdenum-tungsten or niobium-cermet (a composite sintered body of molybdenum and alumina)-tungsten, the sealing of the electrode may be made at the niobium portion and further the niobium portion may be sealed with a frit material so that the frit material covers a part of accurately controlled portion of molybdenum or cermet for protecting the niobium portion. It is thus possible to relax the thermal stress and prevent the corrosion of niobium.

The electrode rod consisting of three kinds of materials creates high production costs and the need for accurate control of the sealing position of the frit material, so that increased production time is required.

According to a luminous container 1A shown in FIG. 2, a cylindrical luminous vessel 2 made of a brittle material functions as an outer supporting body at the end 2a of the luminous vessel, and an inner supporting body 3 made of a brittle material has the analogous shape of a cylinder as the outer supporting body. A clamped portion 8b of the plate-shaped metal piece 8 is clamped and fixed between the luminous container 2 and inner supporting body 3. The plate-shaped

metal piece 8 functions as a supporting member for the current through conductor 5 and electrode 5a. The plate-shaped metal piece may preferably have a seamless and integrated structure for obtaining air-tightness of the luminous vessel.

5 Non-clamped portions 8a and 8c are protruded from the brittle material, and the clamped portion 8b is embedded in the brittle material. Both faces of the clamped portion 8b is pressed as shown in an arrow "A" direction to deform the clamped portion 8b and to relax the stress due to the difference of physical properties of the brittle material and metal. 10 Further, the luminous vessel 2 and inner supporting body 3 directly contact each other at an interface 50 direct under the clamped portion 8b.

FIG. 3 is a cross sectional view schematically showing an

15 HPS type luminous container 42 of a prior art. A curved part 8c is formed between the cover 8a and clamped portion 8b. A hole 8d is formed in the cover 8a for passing the electrode 5a and current through conductor 5. The hole 8d is utilized to supply luminous substances or gas to be sealed into the luminous container, the electrode and current through 20 conductor are then inserted and connected with the cap-like metal piece to assemble the luminous vessel by means of welding, soldering or the like. According to the present example, although the non-clamped portion has a structure of a cover continuously formed from the clamped portion, the 25 shape is not limited and may be appropriately selected depending on the method or state of the connection with the current through conductor.

If molybdenum material having excellent corrosion resistance is used for the cap-like metal piece and current through 30 conductor, the current through conductor and electrode can be formed with two kinds of materials of molybdenum and tungsten. Therefore the requirement to make the current through conductor and electrode of three kinds of materials of niobium-molybdenum-tungsten or niobium-cermet (composite sintered body of molybdenum and alumina)-tungsten is removed. Further the accurate control of the sealed positions with frit material is unnecessary.

Preferably, in FIG. 2, the sintering shrinkage of the luminous vessel 2 as the outer supporting body is made larger than 40 that of the inner supporting body 3. For this, for example shown in FIG. 3, the bodies 2A, 3A to be sintered and plate-shaped metal piece 8 are assembled.

The inner diameter of the body 3A to be sintered for the inner supporting body 3 is designed substantially same as the 45 outer diameter of the current through conductor, so that the positioning accuracy of the electrode can be improved to prevent the corrosion of the side face of the current through conductor and the inner surface of the electrode supporting member. In this case, the diameter of winding part 5a of a 50 tungsten coil at the tip end of the electrode is made larger than the inner diameter of the inner supporting body, so that it may be impossible to insert the electrode from the outside of the luminous container. In this case, the electrode and current through conductor are inserted in the inner space in advance 55 in the assembling stage of the bodies to be sintered for the electrode supporting member and inner supporting body. The bodies 2A, 3A and plate-shaped metal piece 8 may be then assembled.

Specifically, the body 2A to be sintered for the luminous 60 vessel is made of ceramic powder. The ceramic powder may contain an additive such as an organic binder or sintering aid. Further, the body 2A to be sintered may be a molded body of the powder, or the calcined body or dewaxed body of the molded body. It is required, however, that the body to be sintered is shrunken after the sintering process.

The body 3A to be sintered for the inner supporting body is made of ceramic powder or mixture of ceramic powder and

metal powder for cermet. The powder may contain an additive such as an organic binder or sintering aid. Further, the body 3A to be sintered may be a molded body of the powder, or the calcined body or dewaxed body of the molded body. It is required, however, that the body 2A to be sintered has a sintering shrinkage larger than that of the body 3A to be sintered.

The material of the body 3A to be sintered may be selected from materials whose densification is already complete such as a sintered body, single crystal glass or the like.

At the time point of FIG. 3 (a) (before sintering), clearances are formed between the body 2A to be sintered and the electrode supporting member 8 and between the electrode supporting member 8 and the body 3A to be sintered. The clearance between the electrode supporting member 8 and the body 3A to be sintered for the inner supporting body may preferably be made smaller than that of the electrode supporting member and the body to be sintered for the outer supporting body. It is thus possible to adhere the supporting member to the inner supporting body with reference to the position of the inner supporting member having a smaller shrinkage, so that the electrode supporting member is clamped more stably.

The bodies 2A and 3A to be sintered are then sintered to densify them. As shown in FIG. 3 (b) (after the sintering), the luminous vessel 2 and inner supporting body 3 having the smaller diameter are generated. The luminous vessel 2 and inner supporting body 3 directly contact each other along an interface 50 so that they are integrated microstructurally.

During the sintering step, the outer diameter of the resulting sintered body of the body 2A for the outer supporting body is made larger than the inner diameter of sintered body of the body 3A for the inner supporting body, if each of the bodies would have been subjected to sintering alone. It is thus possible to apply a pressing force from the luminous vessel and the inner supporting body to the clamped portion 8b of the electrode supporting member 8 during the sintering, so as to improve the adhesion and air-tightness.

On the viewpoint, the ratio (RO/RI) may preferably be 1.04 or higher and more preferably be 1.05 or higher, provided that "RO" represents the outer diameter of the sintered body obtained by sintering the body for the inner supporting body alone and "RI" represents the inner diameter of the sintered body obtained by sintering the body for the outer supporting body alone.

If "RO/RI" is too larger, cracks tend to be generated in the outer or inner supporting body. On the viewpoint, "RO/RI" may preferably be 1.20 or lower and more preferably be 1.15 or lower.

For example, a knife edge-shaped portion is provided at the tip end of the clamed portion. Alternatively, a C-plane or an R-plane is provided at the tip end of the clamped portion. It is thus possible to improve the wettability of the brittle material and the metal piece at the contact point at the tip end of the clamped portion. When a corner (sharp portion) is left at the tip end of the clamped portion, microcracks may be observed starting from the corner in some samples. However, such cracks are not observed by applying the knife edge, C plane or R plane shape at the tip end of the clamped portion, resulting in a reduction of the stress.

According to the tip end of a luminous container 1B in FIG. 4, on the side of inner surface 2b of the tip end 2a (not shown) of a cylindrical luminous vessel 2 made of brittle material, it is provided a cylindrical outer supporting body 9 having an outer shape of the analogous shape as that of the vessel and made of the same brittle material. An cylindrical inner supporting body 10 is provided inside of the outer supporting body 9. A seamless and cap-like clamped portion 8b of the

plate-shaped metal piece 8A is clamped and fixed between the outer supporting body 9 and inner supporting body 10.

The non-clamped portions 8a and 8c of the electrode supporting member 8 made of the plate-shaped metal piece is protruded from the brittle material and the clamped portion 8b is embedded in the brittle material. Both sides of the clamped portion 8b is pressed toward the radial direction by the brittle material so as to deform the clamped portion 8b and thus to absorb and relax the stress due to the difference of physical property of the brittle material and metal. Further, the outer supporting body 9 and inner supporting body 10 directly contact each other at an interface 50 direct under the clamped portion.

In the case of FIG. 4, the diameter of winding part 5a of a coil made of tungsten or the like at the tip end of the electrode is made larger than the inner diameter of the inner supporting body 10, so that it may be impossible to insert the electrode rod from the outside of the luminous container into the inner space. In this case, the electrode and current through conductor are inserted in the inner space in advance in the assembling stage of the electrode supporting member and inner supporting body. The inner and outer supporting bodies are integrated utilizing the sintering shrinkage of the inner and outer supporting bodies, and the outer supporting body and luminous vessel are integrated utilizing the difference of the sintering shrinkage.

A hole 8d for inserting the current through conductor 5 is formed in the cover portion 8a of the electrode supporting member 8A. The hole, another hole in the inner supporting body and a clearance with the current through conductor are utilized to supply luminous substances or gas to be sealed into the luminous container, and current through conductor is then connected with the electrode supporting member to seal the luminous container by means of welding, soldering or the like in air-tight manner to obtain a luminous container 1B.

By applying the structure as shown in FIG. 4, it can be used a cap-like electrode supporting member 8A having a diameter smaller than the inner diameter of the luminous vessel 2 by the thickness of the outer supporting body 9. Since the inner pressure of the luminous vessel 2 is higher than atmospheric pressure, the diameter of the electrode supporting member 8A may preferably be made smaller so that the stress generated in the electrode supporting member 8A can be advantageously reduced. It is further possible to considerably reduce the contact area of the electrode supporting member 8A and corrosive luminous substance in the inner space 7 to effectively reduce the corrosion of the electrode supporting member 8A.

In the drawings following FIG. 5, parts having the same functions as those shown in FIGS. 2 and 4 are specified by the same numerals and the description may be omitted. According to a luminous container 1C of FIG. 5, a cylindrical luminous vessel 2 made of brittle material functions as the outer supporting body, and the clamped portion 8b of the electrode supporting member 8 is clamped between the inner surface 2b of the luminous vessel 2 and the inner supporting body 10 made of brittle material.

According to the present example, a protrusion 10c is formed in the inner supporting body 10 toward the center of the inner space 7. The inner surface 10b of the protrusion 10c substantially has the same diameter and functions as a guide for protecting the electrode conducting portion 5. The outer surface 10a of the protrusion 10 is shaped to form a curved and inclined face along with the angle of radiation of light to avoid the interference of radiation from the luminous portion. Such protrusion prevents the deformation and corrosion of the electrode conductor 5 due to the luminous substance

## 11

during light luminescence. It is further possible to reduce the volume not utilized for the light luminescence in the luminous vessel to reduce the amount of luminous substance sealed in the luminous vessel.

At the end of a luminous vessel 1D shown in FIG. 6, inside of an outer supporting body 14 made of brittle material, it is provided a cylindrical inner supporting body 15 having the analogous shape and made of the same material as the outer supporting body. The clamped portion 8b of an electrode supporting member 8A composed of a plate-shaped metal piece is clamped and fixed between the outer supporting body 14 and inner supporting body 15. The end of the cylindrical luminous vessel 2 of brittle material is provided outside of the outer supporting body 14 to form a luminous vessel 1D.

According to the present example, protrusions 14a and 15a are formed in supporting bodies 14, 15 toward the center of the inner space, respectively. The inner surface 15b of the protrusion 15a substantially has the same diameter and functions as a guide for protecting the electrode conducting portion 5. The outer surface 14a of the protrusion 14 is shaped to form a curved and inclined face along the angle of radiation of light to avoid the prevention of radiation from the luminous portion. Such protrusions 14a and 15a are provided for preventing the deformation and corrosion of the electrode conducting portion and electrode due to the luminous substance during light luminescence. It is further possible to reduce the volume not utilized for the light luminescence in the luminous vessel to reduce the amount of luminous substance sealed in the luminous vessel.

At the end of a luminous vessel 1E shown in FIG. 7, a cylindrical luminous vessel 2 made of brittle material functions as the inner supporting body, and an outer supporting body 13 made of brittle material has the analogous shape of a cylinder. The clamped portion 8b having the analogous shape as the luminous vessel 2 and outer supporting body 13 is clamped and fixed between the luminous vessel 2 and outer supporting body 13. Non-clamped portions 8a and 8c are protruded from the brittle material and the clamped portion 8b is embedded in the brittle material. The clamped portion 8b is pressed radially of the luminous vessel 2 with the brittle material to deform the clamped portion 8b to absorb and relax the stress due to the difference of physical property of the brittle material and metal. Further, the luminous vessel 2 and outer supporting body 13 directly contact each other along an interface 50 direct under the clamped portion 8b.

A pushing portion 13a is provided at the outer end of the outer supporting body 13 for supporting a cover 8a of an electrode supporting member 8, so that the deformation of 8a due to the inner pressure in the luminous vessel can be prevented.

As in the present example, when the luminous vessel 2 is used as the inner supporting body, the sintering shrinkage of the luminous vessel 2 is made smaller than that of the outer supporting body 13, or the luminous vessel 2 is made of a material not susceptible for sintering shrinkage, as described above.

At the end of a luminous vessel 1F shown in FIG. 8, inside of a cylindrical outer supporting body 16 made of brittle material, it is provided a cylindrical inner supporting body 17 having the analogous shape as the outer supporting body and made of brittle material. The cylindrical clamped portion 8b having the analogous shape as the outer supporting body 16 and inner supporting body 17 is clamped and fixed between the outer supporting body 16 and inner supporting body 17.

## 12

The outer supporting body 16 further clamp the outer surface 2c of the end portion 2a of the cylindrical luminous vessel 2 made of brittle material from the outside to form the luminous container 1F.

5 As in the present example, when the luminous vessel 2 is pressed and clamped with the outer supporting body 16, the sintering shrinkage of the luminous vessel 2 is made smaller than that of the outer supporting body 16, or the luminous vessel 2 is made of a material not susceptible for sintering shrinkage, as described above.

10 As in the present example, when the outer supporting body 16 clamps the clamped portion 8b and the luminous vessel 2 from the outside, the contact area of the electrode supporting member 8 with luminous substance in the inner space can be considerably reduced to further improve the reliability of the end portion.

15 According to a luminous container 1G shown in FIG. 9, inside of a cylindrical outer supporting body 16 made of brittle material, it is provided a cylindrical base 17d of an inner supporting body 17A made of brittle material and having the analogous shape as the outer supporting body. The clamped portion 8b having a cylindrical portion with the analogous shape as the outer and inner supporting bodies between the outer supporting body 16 and inner supporting body 17A. The cylindrical luminous container 2 made of brittle material is provided inside of the outer supporting body 16 to form a luminous vessel.

20 According to the present example, a protrusion 17a is formed in the inner supporting body 17A toward the center of the inner space 7. The inner surface 17c of the protrusion 17a substantially has the same diameter as the current through conductor 5 and electrode 5a, and functions as a guide for protecting the electrode conducting portion 5 and electrode 5a. The outer surface 17b of the protrusion 17a is shaped to 25 form a curved and inclined face along the angle of radiation of light to avoid the interference of irradiation from the luminous vessel. Such protrusion prevents the deformation and corrosion of the electrode conducting portion 5 and electrode 5a due to the luminous substance during light luminescence. 30 It is further possible to reduce the volume not utilized for the light luminescence in the luminous vessel to reduce the amount of luminous substance sealed in the luminous vessel.

35 FIG. 10 shows a luminous container of a prior art.

40 FIGS. 11 to 15 show luminous containers each using so called luminous vessel 2 of elliptical type (one body type).

45 An alumina supporting tube 4 is fixed on the inner surface 12b of each of the ends 12a of a luminous vessel 12 having a shape of a straight tube through a sealing member 3 made of alumina. The supporting tube 4 and current through conductor 5 are sealed with a sealing material 6. According to this structure, luminous substance at high temperature filled in the inner space 7 of the luminous vessel 12 contacts the sealing material 6, so that the corrosion of the sealing material 6 tends 50 to occur to result in a structural problem.

55 Further, although niobium may preferably be applied as the material of the current through conductor 5 having a thermal expansion coefficient near that of a ceramic (alumina), niobium is susceptible to a luminous substance and thus problematic. Therefore, the current through conductor and electrode may be made of three kinds of materials such as niobium-molybdenum-tungsten or niobium-cermet (a composite sintered body of molybdenum and alumina)-tungsten, the sealing of the electrode may be made at the niobium portion and further the niobium portion may be sealed with a frit material so that the frit material covers a part of accurately controlled portion of molybdenum or cermet for protecting

## 13

the niobium portion. It is thus possible to relax the thermal stress and prevent the corrosion of niobium.

The electrode rod consisting of three kinds of materials creates high production costs and the need for accurate control of the sealing position of the frit material, so that increased production time is required.

According to a luminous container 11A shown in FIG. 11, a cylindrical luminous vessel 12 made of a brittle material functions as an outer supporting body at the end 12a of the luminous vessel, and an inner supporting body 19 made of a brittle material has a shape of a cylinder having the analogous shape as the outer supporting body. A clamped portion 8b of the plate-shaped metal piece 8 is clamped and fixed between the luminous container 12 and inner supporting body 19. The plate-shaped metal piece 8 functions as a supporting member for the electrode 5a. Non-clamped portions 8a and 8c are protruded from the brittle material, and the clamped portion 8b is embedded in the brittle material. Both faces of the clamped portion 8b is pressed to deform the clamped portion 8b and to relax the stress due to the difference of physical properties of the brittle material and metal. Further, the luminous vessel 12 and inner supporting body 19 directly contact each other direct under the clamped portion 8b along surface 12b.

8a has a shape of a disk and functions as a cover or a cap. A curved part 8c is formed between the cover 8a and clamped portion 8b. A hole 8d is formed in the cover 8a for passing the electrode 5a and current through conductor 5. The hole is utilized to supply luminous substance or gas to be sealed into the luminous container, the electrode and current through conductor are then inserted and connected with the cap-like metal piece to assemble the luminous vessel by means of welding, soldering or the like.

According to a luminous container 11B shown in FIG. 12, the clamped portion 8b of the electrode supporting member 8 is clamped between the inner surface 12b of the end portion 12a of the luminous vessel 12 and the cylindrical inner supporting body 20, as described above. According to the present example, it forms a cylindrical protrusion 20a having a constant diameter protruding from the inner supporting body 20 toward the center of the inner space 7. The protrusion 20a functions as a guide for protecting the current through conductor 5 and electrode 5a.

According to the tip end of a luminous vessel 11C shown in FIG. 13, the luminous vessel 12 made of brittle material functions as the inner supporting body, and the outer supporting body 13 made of brittle material has the analogous shape as the inner supporting body. The clamped portion 8b having the analogous shape as the luminous vessel 12 and outer supporting body 13 is clamped and fixed between the luminous vessel 12 and outer supporting body 13. The non-clamped portions 8a and 8c are protruded from the brittle material and the clamped portion 8b is embedded in the brittle material. The clamped portion 8b is pressed toward the radial direction in the luminous vessel 12 by the brittle material so as to deform the clamped portion 8b and thus to absorb and relax the stress due to the difference of physical property of the brittle material and metal. Further, the outer supporting body 13 and luminous vessel 12 directly contact each other direct under the clamped portion 12c. A pushing portion 13a is provided at the outer tip end of the outer supporting body 13 for supporting the cover 8a of the electrode supporting member 8 from the outside to prevent the deformation of 8a by the inner pressure of the luminous vessel.

According to the tip end of a luminous vessel 11D shown in FIG. 14, inside of a cylindrical outer supporting body 25 made of brittle material, it is provided a cylindrical inner

## 14

supporting body 23 made of brittle material and having the analogous shape and the same diameter as the outer supporting body. The cylindrical clamped portion 8b having the analogous shape as the outer supporting body 25 and inner supporting body 23 is clamped and fixed between the outer supporting body 25 and inner supporting body 23. The outer supporting body 25 clamps the outer surface 12c of the end portion 12a of the cylindrical luminous vessel 12 made of brittle material from the outside to form a luminous vessel 11D.

A luminous container 11E shown in FIG. 15 is substantially the same as the luminous container 11D of FIG. 14. According to FIG. 15, however, the inner supporting body 23 has a cylindrical protrusion 23a protruding toward the center of the inner space 7. The protrusion 23a functions as a guide for protecting the current through conductor 5 and electrode 5a.

FIG. 16 shows a luminous container of a prior art.

FIGS. 17 to 21 show luminous vessels each using so called luminous vessel 2 of elliptical type (two bodies type).

A tube-like luminous vessel 22 has a shape of a barrel. The current through conductor 5 is sealed with a sealing material 6 at both ends of the luminous vessel 22. Further, although niobium may preferably be applied as the material of the current through conductor 5 having a thermal expansion coefficient near that of a ceramic (alumina), niobium is susceptible to a luminous substance and thus problematic. Therefore, the current through conductor and electrode may be made of three kinds of materials such as niobium-molybdenum-tungsten or niobium-cermet (a composite sintered body of molybdenum and alumina)-tungsten, the sealing of the electrode may be made at the niobium portion and further the niobium portion may be sealed with a frit material so that the frit material covers a part of accurately controlled portion of molybdenum or cermet for protecting the niobium portion. It is thus possible to relax the thermal stress and prevent the corrosion of niobium.

The electrode rod consisting of three kinds of materials creates high production costs and the need for accurate control of the sealing position of the frit material, so that increased production time is required.

According to a luminous container 21A shown in FIG. 17, a cylindrical luminous vessel 22 made of a brittle material functions as an outer supporting body at the end 22a of the luminous vessel, and an inner supporting body 19 made of a brittle material has a shape of a cylinder of the analogous shape as the outer supporting body. A clamped portion 8b of the plate-shaped metal piece is clamped and fixed between the luminous container 22 and inner supporting body 19. The plate-shaped metal piece 8 functions as a supporting member for the current through conductor 5 and electrode 5a. Non-clamped portions 8a and 8c are protruded from the brittle material, and the clamped portion 8b is embedded in the brittle material. Both faces of the clamped portion 8b is pressed to deform the clamped portion 8b and to relax the stress due to the difference of physical properties of the brittle material and metal. Further, the luminous vessel 22 and inner supporting body 19 directly contact each other direct under the clamped portion 8b along surface 22b.

8a has a shape of a disk and functions as a cover or a cap. A curved part 8c is formed between the cover 8a and clamped portion 8b. A hole 8d is formed in the cover 8a for passing the electrode 5a and current through conductor 5. The hole 8d is utilized to supply luminous substances or gas to be sealed into the luminous container, the electrode and current through

## 15

conductor are then inserted and connected with the cap-like metal piece to assemble the luminous vessel by means of welding, soldering or the like.

If molybdenum material having excellent corrosion resistance is used for the cap-like metal piece and current through conductor, the current through conductor and electrode can be formed of two kinds of materials of molybdenum and tungsten. Therefore the requirement to make the current through conductor and electrode of three kinds of materials of niobium-molybdenum-tungsten or niobium-cermet (composite sintered body of molybdenum and alumina)-tungsten is removed. Further the accurate control of the sealed positions with frit material is unnecessary.

According to a luminous container 21B shown in FIG. 18, the clamped portion 8b of the electrode supporting member 8 is clamped between the inner surface 22b of the end portion 22a of the luminous vessel 22 and the cylindrical part 27a of the inner supporting body 27, as described above. According to the present example, it is formed a protrusion 27b protruding in the inner supporting body 27 toward the center of the inner space 7. The protrusion 27b functions as a guide for protecting the current through conductor 5.

At the tip end of a luminous vessel 21C shown in FIG. 19, the luminous vessel 22 made of brittle material functions as the inner supporting body, and the cylindrical outer supporting body 13 made of brittle material has the analogous shape as the inner supporting body. The clamped portion 8b having the analogous shape as the luminous vessel 22 and outer supporting body 13 is clamped and fixed between the luminous vessel 22 and outer supporting body 13. The non-clamped portions 8a and 8c are protruded from the brittle material and the clamped portion 8b is embedded in the brittle material. The clamped portion 8b is pressed toward the radial direction in the luminous vessel by the brittle material so as to deform the clamped portion 8b and thus to absorb and relax the stress due to the difference of physical property of the brittle material and metal. Further, the luminous vessel 22 and outer supporting body 13 directly contact each other direct under the clamped portion 8b along surface 50.

At the tip end of a luminous vessel 21D shown in FIG. 20, inside of a cylindrical outer supporting body 29 made of brittle material, it is provided a cylindrical inner supporting body 30 made of brittle material and having the analogous shape and the same diameter as the outer supporting body. The cylindrical clamped portion 8b is clamped and fixed between the outer supporting body 29 and inner supporting body 30. The outer supporting body 29 clamps the outer surface 22c of the end portion 22a of the cylindrical luminous vessel 22 made of brittle material from the outside to form a luminous vessel 21D. A pushing portion 29a is provided at the outer end portion of the outer supporting body 29 for supporting the cover 8a of the electrode supporting portion from the outside, so that the deformation of 8a due to the inner pressure can be prevented.

A luminous container 21E shown in FIG. 21 is substantially the same as the luminous container 21D of FIG. 20. According to FIG. 21, however, the inner supporting body 30A has a cylindrical protrusion 30a protruding toward the center of the inner space 7. The protrusion 30a functions as a guide for protecting the current through conductor 5 and electrode 5a.

FIG. 22 shows a luminous vessel of a prior art.

FIGS. 23 to 29 show luminous vessels each using so called luminous vessel 32 of elliptical type (one body type).

A tube-like luminous vessel 32 has a shape of a barrel. The current through conductor 5 is sealed with a sealing material 6 at each end of the luminous vessel 32. Further, although

## 16

niobium may preferably be applied as the material of the current through conductor 5 having a thermal expansion coefficient near that of a ceramic (alumina), niobium is susceptible to a luminous substance and thus problematic. Therefore, the current through conductor and electrode may be made of three kinds of materials such as niobium-molybdenum-tungsten or niobium-cermet (a composite sintered body of molybdenum and alumina)-tungsten, the sealing of the electrode may be made at the niobium portion and further the niobium portion may be sealed with a frit material so that the frit material covers a part of accurately controlled portion of molybdenum or cermet for protecting the niobium portion. It is thus possible to relax and the thermal stress and prevent the corrosion of niobium.

The electrode rod consisting of three kinds of materials creates high production costs and the need for accurate control of the sealing position of the frit material, so that increased production time is required.

According to a luminous container 31A shown in FIG. 23, a cylindrical luminous vessel 32 made of a brittle material functions as an outer supporting body at the end 32a of the luminous vessel 32, and a cylindrical inner supporting body 19 made of a brittle material has the analogous shape as the outer supporting body. A clamped portion 8b of the plate-shaped metal piece 8 is clamped and fixed between the luminous container 32 and inner supporting body 19. The plate-shaped metal piece 8 functions as a supporting member for the current through conductor 5 and electrode 5a. Non-clamped portions 8a and 8c are protruded from the brittle material, and the clamped portion 8b is embedded in the brittle material. Both faces of the clamped portion 8b is pressed to deform the clamped portion 8b and to relax the stress due to the difference of physical properties of the brittle material and metal.

According to the present example, the diameter of winding part 5a of a coil made of tungsten or the like at the tip end of the electrode is larger than the inner diameter of the inner supporting body 19, so that the electrode and current through conductor are integrated with the luminous vessel while they are inserted into the hole of the inner supporting body 19 in advance. Since the electrode supporting body and current through conductor are not sealed in air-tight manner, luminous substance is supplied into the luminous vessel through a clearance of the electrode supporting member and current through conductor. They are then sealed in air-tight manner. It is thus possible to complete the assembly of the luminous container.

According to a luminous container 31B shown in FIG. 24, the clamped portion 8b of the electrode supporting member 8 is clamped between the inner surface 32b of the end portion 32a of the luminous vessel 32 and the inner supporting body 30A, as described above. According to the present example, it forms a protrusion 30a in the inner supporting body 30A toward the center of the inner space 7. The protrusion 30a functions as a guide for protecting the current through conductor 5 and electrode 5a.

At the tip end of a luminous vessel 31C shown in FIG. 25, the luminous vessel 32 made of brittle material functions as the inner supporting body, and the cylindrical outer supporting body 13 made of brittle material has the analogous shape as the inner supporting body. The clamped portion 8b is clamped and fixed between the luminous vessel 32 and outer supporting body 13. The non-clamped portions 8a and 8c are protruded from the brittle material and the clamped portion 8b is embedded in the brittle material. The clamped portion 8b is pressed toward the radial direction by the brittle material so

as to deform the clamped portion  $8b$  and thus to absorb and relax the stress due to the difference of physical property of the brittle material and metal.

At the tip end of a luminous vessel  $31D$  shown in FIG. 26, inside of a cylindrical outer supporting body  $29$  made of brittle material, it is provided a cylindrical inner supporting body  $30$  made of brittle material and having the analogous shape and the same diameter as the outer supporting body. The cylindrical clamped portion  $8b$  having the analogous shape as the outer supporting body  $29$  and inner supporting body  $30$  is clamped and fixed between the outer supporting body  $29$  and inner supporting body  $30$ . The outer supporting body  $29$  clamps the outer surface  $32c$  of the end portion  $32a$  of the cylindrical luminous vessel  $32$  made of brittle material from the outside to form a luminous vessel  $31D$ .

A luminous container  $31E$  shown in FIG. 27 is substantially the same as the luminous container  $31D$  of FIG. 26. According to FIG. 27, however, the inner supporting body  $30A$  has a cylindrical protrusion  $30a$  protruding toward the center of the inner space  $7$ . The protrusion  $30a$  functions as a guide for protecting the current through conductor  $5$  and electrode  $5a$ .

A luminous container  $31F$  shown in FIG. 28 is substantially the same as the luminous container  $31B$  of FIG. 24. According to FIG. 28, however, the distance of opposing electrodes is smaller and the inner supporting body  $30A$  has a longer cylindrical protrusion  $30a$  protruding toward the center of the inner space  $7$ . The protrusion  $30a$  functions as a guide for protecting the current through conductor  $5$  and electrode  $5a$ .

A luminous container  $31G$  shown in FIG. 29 is substantially the same as the luminous container  $31E$  of FIG. 27. According to FIG. 29, however, the inner supporting body  $30A$  has a longer and cylindrical protrusion  $30a$  protruding toward the center of the inner space  $7$ . The protrusion  $30a$  functions as a guide for protecting the current through conductor  $5$  and electrode  $5a$ . A pushing portion  $29a$  is provided at the outer end portion of the outer supporting body  $29$  for supporting the cover  $8a$  of the electrode  $8$  from the outside to prevent the deformation of  $8a$  due to the inner pressure of the luminous vessel.

FIG. 30 shows a luminous container of a prior art.

FIGS. 31 to 34 show luminous vessels for high pressure discharge lamps of so called HPS type.

A current through conductors  $5$  are supported through a plug  $40$  made of alumina on the inner surface  $42b$  of a straight tube-shaped luminous vessel  $42$  at both ends  $42$ , respectively. The conductor  $5$  and plug  $40$  are sealed with sealing material  $6$ .

According to a luminous container  $41A$  shown in FIG. 31, a cylindrical luminous vessel  $42$  made of a brittle material functions as an outer supporting body at the end  $42a$  of the luminous vessel  $42$ , and an inner supporting body  $19$  made of a brittle material has the analogous shape as the outer supporting body. A clamped portion  $8b$  of the plate-shaped metal piece  $8$  is clamped and fixed between the luminous container  $42$  and inner supporting body  $19$ . The plate-shaped metal piece  $8$  functions as a supporting member for the current through conductor  $5$  and electrode  $5a$ . Non-clamped portions  $8a$  and  $8c$  are protruded from the brittle material, and the clamped portion  $8b$  is embedded in the brittle material. Both faces of the clamped portion  $8b$  is pressed to deform the clamped portion  $8b$  and to relax the stress due to the difference of physical properties of the brittle material and metal. The luminous vessel  $42$  and inner supporting body  $19$  directly contact each other direct under the clamped portion  $8b$  along surface  $50$ .

At the tip end of a luminous vessel  $41B$  shown in FIG. 32, on the side of the inner surface  $42b$  of the end portion  $42a$  of a cylindrical luminous vessel  $42$  made of brittle material, a cylindrical outer supporting body  $9$  made of the same brittle material is provided. A cylindrical inner supporting body  $10$  is provided inside of the outer supporting body  $9$ . The clamped portion  $8b$  of a cap-like plate-shaped metal piece  $8A$  is clamped and fixed between the outer supporting body  $9$  and inner supporting body  $10$ .

Non-clamped portions  $8a$  and  $8c$  of the electrode supporting body  $8A$  composed of a plate-shaped metal piece are protruded from the brittle material, and the clamped portion  $8b$  is embedded in the brittle material. Both faces of the clamped portion  $8b$  is pressed by the brittle material radially to deform the clamped portion  $8b$  and to relax the stress due to the difference of physical properties of the brittle material and metal. The outer supporting body  $9$  and inner supporting body  $10$  directly contact each other direct under the clamped portion along surface  $50$ .

According to a luminous container  $41C$  shown in FIG. 33, a cylindrical luminous vessel  $42$  made of a brittle material functions as an outer supporting body, and the clamped portion  $8b$  of the electrode supporting member  $8$  is clamped between the inner surface  $42b$  of the luminous vessel  $42$  and the inner supporting body  $10$  made of brittle material.

According to the present example, a protrusion  $10a$  is formed in the inner supporting body  $10$  toward the center of the inner space  $7$ . The inner surface  $10b$  of the protrusion  $10a$  substantially has the same diameter and functions as a guide for protecting the electrode conducting portion  $5$  and electrode  $5a$ . The outer surface  $10a$  of the protrusion  $10$  is shaped to form a curved and inclined face along the angle of radiation of light to avoid the interference of the radiation from the luminous vessel. Such protrusion prevents the deformation and corrosion of electrode conducting portion  $5$  due to the luminous substance during light luminescence. It is further possible to reduce the volume not utilized for the light luminescence in the luminous vessel and to reduce the amount of luminous substance sealed in the luminous vessel.

According to the present example, the diameter of winding part  $5a$  of a coil made of tungsten or the like at the tip end of the electrode is larger than the inner diameter of the inner supporting body  $10$ , so that the electrode and current through conductor are integrated with the luminous vessel while they are inserted into the hole of the inner supporting body  $10$  in advance. Since the electrode supporting member and current through conductor are not sealed in air-tight manner, luminous substance is supplied into the luminous vessel through a clearance of the electrode supporting member and current through conductor. They are then sealed in air-tight manner. It is thus possible to complete the assembly of the luminous container.

At the tip end of a luminous vessel  $41D$  shown in FIG. 34, inside of a cylindrical outer supporting body  $43$  made of brittle material, a cylindrical inner supporting body  $44$  made of the same brittle material is provided. The clamped portion  $8b$  of an electrode supporting member  $8A$  composed of a plate-shaped metal piece is clamped and fixed between the outer supporting body  $43$  and the cylindrical part  $44a$  of the inner supporting body  $44$ . The end portion  $42a$  of a cylindrical luminous vessel  $42$  made of brittle material is further provided outside of the outer supporting body  $43$  to assemble a luminous container  $41D$ .  $42c$  represents an edge of the outer supporting body.

According to the present example, a protrusion  $44b$  is formed toward the center of the inner space  $7$  in the supporting body  $44$ . The inner surface of the protrusion  $44b$  has a

substantially constant diameter and functions as a guide for protecting the current through conductor 5 and electrode 5a.

According to the present invention, an adhesive may also be used on the outside of the electrode supporting member composed of a plate-shaped metal piece. Although the kind of the adhesive is not particularly limited, so called frit glass is preferred, and a glass composition of Al<sub>2</sub>O<sub>3</sub>-Dy<sub>2</sub>O<sub>3</sub>-SiO<sub>2</sub> system and that further containing nitrogen atom are most preferred.

When the luminous vessel is made of sapphire (alumina single crystal) or translucent alumina material consisting mainly of sapphire, the longitudinal axis of the tube shaped luminous vessel corresponds to the c-axis of sapphire. It is preferred that the tube axis of the luminous vessel and the c-axis are intersected at an angle of 10° or lower. It is thus possible to considerably reduce the incidence of cracks in sapphire along and near the interface between the luminous vessel and the inner or outer supporting body fixed at the end of the luminous vessel, because the distribution of the thermal stress may be made symmetrical with respect to the axis. On the viewpoint, the angle of the c-axis of sapphire forming the luminous vessel and the tube axis of the luminous vessel may more preferably be 5° or lower.

Further, the electrode supporting member composed of the plate-shaped metal piece may substantially have a shape of a cap, as described above. Such cap may be produced by drawing or the like, although the production method is not particularly limited. However, if drawing process is applied for processing a rolled body for example, embrittlement may progress during the heat treatment in a direction perpendicular to the direction of rolling. Attention is required on this point during the drawing process. Variations of the metal members may be appropriately adjusted depending on the design of the bonded body.

For example, at the air-tight sealing part at the end portion of a high pressure sodium lamp, Nb or the like can be used. If a soft metal such as Nb is used, the thickness of the metal is designed to be thicker for avoiding the deformation under high pressure. It is further considered to provide a pushing part (of brittle material portion) for avoiding the over deformation of metal due to high pressure and temperature. However, the sintering is needed to be performed under inert atmosphere (including vacuum) for preventing the embrittlement of Nb.

When an Nb thin plate and Nb current conductor are used, the sealing may be performed by pressure bonding or mechanical sealing such as fitting (so called, guillotine method). When the metal part of the bonded body is near an auxiliary electrode (winding, printing by metalizing) on the outer surface of a luminous vessel, it is necessary to provide an insulating means for preventing shortage near the metal part of the bonded body. Alternatively, on the contrary, an appropriate electrical circuit may be provided in the metal part and auxiliary electrode portion.

When the luminous vessel is made of quartz, sintered quartz may be used for the outer supporting body. After the sintering, it may be necessary to apply a technique of reducing foams (the atmosphere may most preferably be vacuum, although reducing atmosphere may be used). Further, the outer supporting body may be made of quartz glass softened by heating at high temperature for press bonding from the outside and sealing.

In the case of a ceramic metal halide lamp in general, the shape of a luminous vessel is divided into a part for inserting an electrode of the luminous vessel and a luminous main portion having a larger diameter. The inventive bonded portion may preferably be used as the end portion of a narrower

tube part, so that a frit sealing structure can be alleviated to improve the heat resistance and the bonded portion (sealing portion) can be used at a higher temperature region, compared with a prior art. As a result, although an elongate narrower part has been necessary for lowering the temperature by drawing thermal flux in a prior design, such capillary may be omitted or the length may be made smaller according to the present invention to provide a compact luminous vessel. The design of an outer lamp may be selected among wider variations and the functionality and appearance can be made excellent. The amount of luminous substance can be reduced to manufacture the luminous vessel more economically.

Further, when a high level of current is supplied into the electrode during on-time in a prior art, a large amount of heat would be generated in the current through conductor sealed with a frit. The temperature of the current through conductor is thus elevated to which generates thermal stress due to the difference of thermal expansion of the frit and alumina and results in cracks in the frit sealing part.

On the contrary, according to the present invention, the current through conductor does not directly contact ceramic material having the different thermal expansion coefficient which avoids thermal stress between the current through conductor and the ceramic material even when a large current is applied to the electrode. The heat generated in the current through conductor due to the supply of the large current is conducted to the thin electrode supporting member, then dispersed in the clamped portion embedded in brittle material and absorbed into the brittle material. The stress generated in the process is smaller than that generated in the prior frit sealed part. Even when a large stress would be generated, such stress can be absorbed with a very small deformation of the clamped portion embedded in the brittle material. It becomes thus possible to supply a large current during on-time or select the wire diameter of the current through conductor without particular limitations.

In the case of a ceramic halide lamp for an automobile, the end portion not contributing to the luminescence is needed to be made smaller. Further, the size of the luminous vessel may be preferably be smaller for reducing the overall thermal capacity. On the side of a circuit for supplying electric power, the size of the luminous vessel can be lowered so that the luminescence (temperature) of the vessel can respond with respect to the power input in a short time to remove the need for excessive starting power. At the same time, it means that the temperature distribution in the luminous vessel can be reduced. That means that unnecessary thermal stress on a ceramic material against thermal shock can be avoided which results in improvement of the reliability of the luminous vessel. For example, high strength PCA luminous vessel material may be advantageously applied for reducing the size of the luminous vessel. PCA has a very small average grain diameter (for example 10 µm or smaller) even after the sintering so as to result in a high strength of 2 or more times of that of the vessel made of a conventional material.

Although the vessel may be produced by means of methods not particularly limited, methods using an inner core such as gel cast molding are preferred, because the inner shape of the luminous vessel can be selected without limitation. Further, when ceramic materials which can be sintered at a low temperature is used for the luminous vessel or outer ring, the embrittlement of the metal part can be prevented to provide the luminous vessel with excellent reliability. The luminous substances may be composed of different kinds of rare earth elements other than prior Sc—Na system in response to the corrosion state of the ceramic vessel.

Further, in the luminous vessel, when Mo or Nb is used for the current through conductor or electrode supporting portion, the turning-on without an outer lamp is difficult. In the case of no outer lamp, coating the surface with a thin metal film may be applied as the solution. The coating with glass or like may be also applied. In the case of metal coating, it is necessary to prevent the exposure of Mo to air due to the interdiffusion of metals. In the case of mercury-free luminous vessel, the metal part of Pt system may be used. The turning-on without an outer lamp in air is possible in the case of pure Pt. Further, a small clearance may be provided between the inner diameter of the (inner) ceramic tube positioned near the electrode inserting part and the inserted electrode for preventing the blacklash of the electrode assembly and for improving the positioning accuracy of the electrode.

Further, when a welded part is distant from the pressure bonded part, fine welding such as laser welding is not necessary this widens the range of welding means. Further, when the metal portion is not cap-shaped, the pipe-shaped portion of the metal member may be welded with the bottom plate part. Further, the bottom plate part and electrode may be welded in advance and then welded with the metal pipe-shaped part.

Further, when the electrode is to be conducted with an outer lead, it is possible to assure the conduction through a part (laterally) other than the direction of the tube axis, because the metal member as well as the electrode are made of a conductor. Further, in addition to the welding, soldering and mechanical fitting, the conduction may be assured by elongating a part of the plate-shaped metal piece to the outside for use as a part of a lead. Further, a part of the plate-shaped metal piece is bent as "U" character for functioning as a part for absorbing the shock and thermal expansion from the outside in use. As described above, the conducting part may be designed without limitation to provide excellent functionality and appearance.

The method of manufacturing the luminous vessel is not particularly limited. The shell portion of the luminous vessel may be molded by (1) extrusion, slurry casting or injection molding so that two parts for the luminous vessel is molded separately, and the molded bodies may be joined before the dewaxing and sintered to integrate them. Further, the shell part of the luminous vessel may be molded (2) by means of lost wax process such as gel cast molding to provide an end portion sealing structure whose design of the shell part is not limited.

Further, in a metal halide lamp, Mo, W, Re or the like has been used on the viewpoint of corrosion resistance. In a high pressure sodium lamp, Nb may be applied for the metal member. Further, as described above, Nb may be applied in a super high pressure mercury lamp.

The luminous bodies may be sealed as follows to provide a discharge lamp.

(1) Metal Halide Lamp (Illumination for General Lighting)

Hg (not essential component), the iodide of a metal (Na, rare earth element or the like) are supplied through a hole of a metal cap (metal cap itself may have a guiding part) made of Mo in Ar atmosphere of 50 to 200 mbar and Mo or W electrode is then inserted and sealed by welding such as TIG welding or laser welding.

(2) Metal Halide Lamp (Automobile Use, Point Light Source)

Metal iodide and Hg (not essential component) are sealed as described in (1). 7 to 20 bar of Xe is used as a starter gas depending on the conditions. Particularly in the case of the present invention, it is possible to completely prevent the evaporation of luminous substances such as a starter gas,

because the sealing can be completed in a very short time and at a low temperature. The material of the shell part may be conventional translucent alumina and may preferably be YAG, sapphire, polycrystalline alumina having a grain diameter of 10  $\mu\text{m}$  or smaller or the like having a high linear transmittance.

(3) High Pressure Na Lamp

Nb is used for the metal cap. The electrode is made of Mo, W or Nb welded with each other. The luminous substance may be Na—Hg amalgam and a starter gas such as Ar or the like or Xe in the case of no Hg used. Particularly when an auxiliary electrode is used on the surface of the tube (irrespective of the kind of the electrode such as coil winding, printing by metallizing or the like), an insulating means may be provided on the auxiliary electrode depending on the cases for preventing the shortcut of the electrode supporting member or the like and auxiliary electrode.

(4) Super High Pressure Mercury Lamp

The material of the shell part may preferably be YAG, sapphire or polycrystalline alumina having a grain diameter of 10  $\mu\text{m}$  or lower having a high linear transmittance. The luminous substances include Hg and Br. Nb as well as Mo and W may be used for the metal cap, and the welding method is the same as described above.

The discharge lamp obtained according to the procedures described above may be turned on by means of an appropriate igniter or ballast.

According to each of the first, second and third aspects of the present invention, a coating composed of a metal or mixture of a metal and ceramics may be provided on the outer surface of the luminous vessel as an optical masking means. The masking means a shading film. For example, in the case of a head lamp for automobile, a shading film is provided on the outer surface of the luminous vessel for controlling the direction of the light, so that the lamp of the opposing automobile does not cause glare (for example for preventing the light directed toward UPPER direction). Such light shading film is disclosed in Japanese Patent publications 2004-149640A, 2004-163911A and 2004-134219A.

A metal forming the shading film is not particularly limited, and may preferably be a metal selected from the group consisting of tungsten, molybdenum, rhenium or the alloys thereof. Further, when mixture of a metal and ceramics is used, the ceramics may preferably contain a constituent of the luminous vessel. Such ceramics was described above as the materials of the luminous vessel. Further, the shading film may be made by applying paste.

## EXAMPLES

### Example 1

A luminous vessel 1A shown in FIG. 2 was produced.

Specifically, a molybdenum plate was subjected to deep drawing to produce a cap-shaped electrode supporting member 8. A cover 8a had a diameter of 2 mm and a thickness of 200  $\mu\text{m}$ . Further, the electrode supporting member had a cylindrical portion having a length of 3 mm and a clamped portion having a thickness of 100  $\mu\text{m}$ . At the curved portion 8c, the thickness was gradually reduced toward the clamped portion. The tip end of the clamped portion 8b has a shape of a wedge. A through hole 8d having a diameter of 500  $\mu\text{m}$  is formed in the cover portion 8a.

Prepared was a tube 3 made of high purity alumina and having an outer diameter of 2 mm, an inner diameter of 0.6 mm and a length of 5 mm which may be inserted inside of the

23

electrode supporting member 8. The tube was used as an inner supporting body and covered with the electrode supporting member 8.

Prepared was a tube-shaped molded body 2 (molded at a pressure of 1500 kg/cm<sup>2</sup>) for luminous vessel, molded with a dry bag molding machine, made of high purity alumina and having an inner diameter of 2.1 mm, an outer diameter of 4 mm and a length of 20 mm. The molded body 2 was used as an outer supporting body. As shown in FIG. 3 (a), the inner supporting body 3 covered with the electrode supporting member 8 was inserted into each side of the molded body for luminous vessel to provide an assembly, which was then sintered in hydrogen atmosphere at 1800° C. to produce a luminous container (FIG. 3 (b)).

### Example 2

A structure shown in FIG. 4 was produced.

Specifically, a molybdenum plate was subjected to deep drawing to produce a cap-shaped electrode supporting member 8A. A cover portion 8a had a diameter of 2 mm and a thickness of 200 mm. Further, the electrode supporting member has a cylindrical portion having a length of 3 mm and a clamped portion 8b having a thickness of 100 µm. At the curved portion 8c, the thickness was gradually reduced toward the clamped portion. The tip end of the clamped portion 8b had a shape of a wedge. A through hole 8d having a diameter of 500 µm was formed in the cover portion 8a.

Prepared was a tube-shaped molded body 10 made of high purity alumina and having an outer diameter of 2 mm, an inner diameter of 0.6 mm and a length of 5 mm which can be inserted inside as the electrode supporting member 8A. The inner molded body 10 was covered with the electrode supporting member 8A. Further, the inner diameter of the inner supporting body 10 is smaller than the diameter of the wound portion 5a of a tungsten coil at the tip end of the electrode, so that the current through conductor 5 and electrode 5a cannot be inserted into the luminous vessel from the outside. The current through conductor 5 (with a diameter of 0.5 mm and the tip end portion has a diameter of 0.8 mm) was inserted into the electrode supporting member in advance.

Prepared was a tube-shaped molded body (molded at a pressure of 1000 kg/cm<sup>2</sup>) molded with a press machine, made of high purity alumina and having an inner diameter of 2.1 mm, an outer diameter of 15 mm and a length of 6.5 mm. The molded body was used as an outer supporting body 9. The inner supporting body 10 assembled with the metal cap and current through conductor and electrode was inserted into the tube-shaped molded body to produce an assembly, which was then sintered in hydrogen atmosphere at 1750° C. to produce a part for fixing electrode of a luminous vessel with the current through conductor and electrode inserted therein in advance. The diameter of the finished part was 12 mm in outer diameter and 5 mm in length. The cylindrical clamped portion 8b of the electrode supporting member 8A was pressed and fixed with the outer supporting body 9 of alumina and inner supporting body 10. The cover portion 8a of the electrode supporting member 8A was exposed to the end of the supporting body as the non-clamped portion. An end part was thus obtained.

Further prepared was a tube-shaped molded body 2 (molded at a pressure of 1500 kg/cm<sup>2</sup>) molded with a dry bag molding machine, made of high purity alumina and having an inner diameter of 12.5 mm, an outer diameter of 15.5 mm and a length of 50 mm. The end part was inserted into each side of the molded body to provide an assembly, which was then sintered in hydrogen atmosphere at 1800° C. to produce a

24

luminous container. FIG. 4 shows an assembly for luminous container having the electrode and current through conductor inserted therein.

### Example 3

A luminous vessel 1C shown in FIG. 5 was produced.

Specifically, an electrode supporting member 8 was prepared according to the same procedure as the example 1. However, the diameter of the electrode supporting member 8 was 4 mm, the length of the cylindrical portion was 4 mm, the thickness of the cover portion 8a was 200 µm, and the thickness of the clamped portion 8b was 100 µm. A hole 8d having a diameter of 500 µm was formed in the cover portion 8a.

Prepared was a tube made of high purity alumina and having a whole length of 10 mm was prepared. The tube has a protrusion 10a having a cylindrical base with an outer diameter of 4 mm, an inner diameter of 0.6 mm and a length of 5 mm and a part whose outer diameter was gradually lowered toward the direction of the length. The tube was used as the inner supporting body 10. The inner supporting body 10 was covered with the electrode supporting member 8.

Prepared was a tube-shaped molded body 2 (molded at a pressure of 1500 kg/cm<sup>2</sup>), molded with a dry bag molding machine, made of high purity alumina and having an inner diameter of 4.2 mm, an outer diameter of 7 mm and a length of 45 mm. The molded body was used as an outer supporting body 2. The inner supporting body 10 covered with the electrode supporting member 8 was inserted into each side of the molded body 10 to provide an assembly, which was then sintered in hydrogen atmosphere at 1800° C. to produce a luminous container.

FIG. 5 also shows a luminous vessel with the current through conductor 5 and electrode 5a inserted therein.

The protrusion 10c of the inner supporting body 10 having the above shape supports the side face of a substantial portion of the current through conductor 5, so that the positioning error of the electrode axis was small, the dimensional accuracy of the distance between the electrodes was excellent and the corrosion due to luminous substance corrosive to the current through conductor and electrode can be reduced. Further, it is expected that the inner volume of the luminous vessel can be reduced and the weight of the luminous substance sealed in the luminous vessel can be reduced.

### Example 4

A luminous container 1D shown in FIG. 6 was produced.

Specifically, it was prepared an electrode supporting member 8A having the same dimensions and shape as those of the example 1.

A tube composed of a high purity alumina sintered body having an outer diameter of 2 mm, an inner diameter of 0.6 mm and a length of 10 mm was prepared and used as the inner supporting body 15. The inner supporting body 15 was covered with the electrode supporting member 8A.

A molded body made of high purity alumina having the whole length of 12.5 mm with a 6.5 mm portion in length having an inner diameter of 2.1 mm and an outer diameter of 15 mm and a tapered portion whose outer diameter was gradually reduced. The molded body was used as an outer supporting body 14. The inner supporting body 15 covered with a metal cap was inserted to provide an assembly, which was then sintered at 1750° C. in hydrogen atmosphere to produce a part for fixing the electrode and current through conductor of a luminous vessel. According to the finished dimensions, the portion had an outer diameter of 12 mm had

a length of 5 mm, and a protrusion whose outer diameter was reduced and tapered had a whole length of 10 mm. The cylindrical portion of the electrode supporting member **8** was used as the clamped portion **8b** pressed and fixed with the outer and inner supporting bodies of alumina. An end part was thus obtained whose cover portion **8a** of the electrode supporting member **8** was exposed to the end of the supporting body as the non-clamped portion.

Further prepared was a tube-shaped molded body (at a molding pressure of 1500 kg/cm<sup>2</sup>) molded by a dry bag molding machine, made of high purity alumina and having an inner diameter of 12.5 mm, an outer diameter of 15.5 mm and a length of 50 mm. The end part was inserted into each of the ends of the molded body **2** to produce an assembly, which was then sintered at 1800° C. in hydrogen atmosphere to produce a luminous container **1D**. FIG. 6 further shows the luminous container with the current through conductor **5** and electrode **5a** inserted therein.

The protrusions **14a** and **15a** composed of the inner and outer supporting bodies support the side face of a substantial portion of the current through conductor **5**. It is thus possible to reduce the positioning error of the electrode axis, to improve the dimensional precision of the distance between the electrodes, and to reduce the corrosion of the current through conductor by corrosive luminous substance. It is further expected that the content of the luminous vessel and the weight of the luminous substance sealed in the luminous vessel can be reduced.

By applying the structure as shown in FIG. 6, it can be used a cap-like electrode supporting member **8A** having a diameter smaller than the inner diameter of the luminous vessel **2** by the thickness of the outer supporting body **14**. Since the inner pressure of the luminous vessel **2** is higher than atmospheric pressure, the diameter of the electrode supporting member **8A** may preferably be made smaller so that the stress generated in the electrode supporting member **8A** can be advantageously reduced. It is further possible to considerably reduce the contact area of the electrode supporting member **8A** and corrosive luminous substance in the inner space **7** to effectively reduce the corrosion of the electrode supporting member **8A**.

#### Example 5

A luminous vessel **1E** shown in FIG. 7 was produced. Specifically, the electrode supporting member **8** having the same dimension and shape as those in the example 1 was prepared.

Prepared was a translucent alumina luminous vessel (made of alumina single crystal such as sapphire), which can be inserted into the electrode supporting member **8**, having an outer diameter of 2 mm, an inner diameter of 0.6 mm and a length of 20 mm. The vessel was used as the inner supporting body which was covered with the electrode supporting member **8**.

Prepared was a ring-shaped molded body (molded at a pressure of 1000 kg/cm<sup>2</sup>) molded with a press molding machine, made of high purity alumina and having an inner diameter of 2.1 mm, an outer diameter of 6 mm and a length of 6.5 mm. The molded body was used as an outer supporting body **13**. Each end portion of the luminous vessel **2** covered with the electrode supporting member was covered with the outer supporting body **13** to provide an assembly, which was sintered at 1800° C. in hydrogen atmosphere to produce a luminous container. FIG. 7 further shows the luminous container with the current through conductor **5** and electrode **5a** inserted therein.

#### Example 6

A luminous vessel **1F** shown in FIG. 8 was produced. Specifically, the electrode supporting member **8A** having the same dimension and shape as those in the example 1 was prepared.

Prepared was a tube made of high purity alumina sintered body and having an outer diameter of 2 mm, an inner diameter of 0.6 mm and a length of 5 mm. The tube was used as the inner supporting body **17** which was covered with the electrode supporting member **8A**.

In addition, an outer supporting body **16** was molded by a press molding machine. The molded body had a base portion **16a** and a protrusion **16b**. The protrusion **16b** had an inner diameter of 2.1 mm and a length of 6.5 mm. The molded body **16** (molded at a pressure of 1000 kg/cm<sup>2</sup>) was made of high purity alumina. The molded body **16** was used as an outer supporting body. The base portion **16a** covered the inner supporting body **17** which was covered with the electrode supporting member **8A**. A translucent alumina tube **2** (mainly consisting of alumina single crystal such as sapphire) having an outer diameter of 4 mm, a thickness of 1 mm and a length of 20 mm was inserted into the protrusion **16b** to produce an assembly, which was then sintered at 1800° C. in hydrogen atmosphere to produce a luminous container. FIG. 8 further shows the luminous container with the current through conductor **5** and electrode **5a** inserted therein.

#### Example 7

A luminous vessel **1G** shown in FIG. 9 was produced.

Specifically, an electrode supporting member **8A** having the same dimensions and shape as those of the example 1 was prepared according to the same procedure as the example 1.

Prepared was an inner supporting body **17A** of high purity alumina which can be inserted into the electrode supporting member **8A**. The inner supporting body **17A** was composed of a high purity alumina sintered body (of a purity of 99.9 percent) having a base portion **17d** with an outer diameter of 2 mm, an inner diameter of 0.6 mm and a length of 5 mm and a protrusion **17a** with a length of 5 mm whose outer diameter is gradually reduced from 2 mm toward the tip end. The inner supporting body **17A** was covered with a metal cap **8A**.

In addition, an outer supporting body **16** was prepared with a press molding machine. The outer supporting body **16** has a base portion **16a** with an inner diameter of 2.1 mm and a length of 6.5 mm and a protrusion **16b** with an inner diameter of 4.1 mm and a length of 6.5 mm. The molded body **16** made of high purity alumina was prepared (molded at a pressure of 1000 kg/cm<sup>2</sup>) and was used as an outer supporting body, into which the inner supporting body **17A** was covered with the electrode supporting member **8A** and was inserted. A translucent alumina luminous vessel **2** (mainly consisting of alumina single crystal such as sapphire) with an outer diameter of 4 mm, a thickness of 1 mm and a length of 20 mm was inserted into the protrusion **16b** to provide an assembly, which was then sintered in hydrogen atmosphere at 1800° C. to produce a luminous container. FIG. 9 also shows the luminous container with the current through conductor **5** and electrode **5a** inserted therein.

The protrusion **17a** of the inner supporting body having the above shape supports the side face of a substantial portion of the current through conductor, so that the positioning error of the electrode axis was small, the dimensional accuracy of the distance between the electrodes was excellent and the corrosion due to luminous substance corrosive to the current through conductor can be reduced. Further, it is expected that

the inner volume of the luminous vessel can be reduced and the weight of the luminous substance sealed in the luminous vessel can be reduced. By applying the structure as shown in FIG. 9, it can be used a cap-like electrode supporting member 8A having a diameter smaller than the inner diameter of the luminous vessel 2 by the thickness of the outer supporting body 16. Since the inner pressure of the luminous vessel 2 is higher than atmospheric pressure, the diameter of the electrode supporting member 8A may preferably be made smaller so that the stress generated in the electrode supporting member 8A can be advantageously reduced. It is further possible to considerably reduce the contact area of the electrode supporting member 8A and corrosive luminous substance in the inner space of the luminous vessel to effectively reduce the corrosion of the electrode supporting member 8A.

The advantageous effects of the present sealing structure will be described below.

(1. Example of Reducing the Deviation of the Sealing Article: in the Case of Sealing a High Pressure Luminous Substance for Automobile Use or the Like)

A ceramic luminous container of a prior art (frit seal) of 35 W and luminous containers of the examples 1 to 7 each having the same watt number were subjected to a test of sealing Xe corresponding to 15 bar. Xe was condensed at a low temperature. n=100 sealing articles were broken in a vacuum container at room temperature having a specific volume for each of the examples and the inner pressure (partial pressure of Xe) of each container was measured for the evaluation.

As a result, according to the article of a prior art, the average of n=100 was 8 atoms. On the contrary, when each of the luminous containers of the examples 1 to 7 was used, the average corresponded to 14.5 atoms.

(2. Air-Tightness of Sealing)

n=30 of the sealed luminous vessels according to each of the examples 1 to 7 were vacuum sealed in a quartz tube and held at 900° C. for 48 hours. A Tesla coil was then used to generate discharge in the tube. "NG" was assigned when luminescence was observed in a quartz outer lamp, and "OK" was assigned when luminescence was not observed in the outer lamp. According to the article of a prior art, n=25/30 were assigned as "NG", In the case of each of the luminous containers of the examples 1 to 7, no "NG" articles were observed in each example.

(Examples of Providing a Masking Material)

In each of the luminous containers of the examples 1 to 7, a shade film functioning as a masking material was formed on a predetermined position of the outer surface of the luminous vessel. Specifically, the luminous vessel was made of translucent alumina. The paste composition was made W/alumina of 60/40 volume percent. 2 to 10 weight percent of ethyl cellulose and an appropriate amount of butyl carbitol acetate were added as binders to the paste to obtain viscous paste. The paste was applied onto the dewaxed calcined body of each example described earlier and dried at 90° C. for 2 hours, and then sintered simultaneously with the luminous vessel. The masking material realized optional light control design.

The invention claimed is:

1. A luminous container comprising an electrode supporting member comprising a pipe-shaped metal piece, a tube-shaped outer supporting body comprising a brittle material, and a pipe-shaped inner supporting body comprising a brittle material and provided inside of said outer supporting body, said piped-shaped metal piece comprising a clamped portion provided between and pressed with said outer and inner supporting bodies and a non-clamped portion not clamped with said outer and inner supporting bodies,

wherein a stress generated along an interface where said clamped portion and each of said outer and inner supporting bodies contact each other is relaxed by deformation of said clamped portion of said pipe-shaped metal piece, and

5 10 15 wherein said outer supporting body and said clamped portion directly contact each other, said clamped portion and said inner supporting body directly contact each other and said outer supporting body and inner supporting body directly contact each other throughout an entire circumference of the inner supporting body.

2. The luminous container of claim 1, wherein said tube-shaped outer supporting body is a luminous vessel.

3. The luminous vessel of claim 2, wherein said inner supporting body has a thickness lowering toward the center of said luminous vessel.

4. The luminous container of claim 1, further comprising a luminous vessel joined to said outer supporting body.

5. The luminous container of claim 4, wherein said outer supporting body is clamped outside of said luminous vessel.

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910

29

20. A luminous container for a high pressure discharge lamp, comprising said luminous container of claim 1, and an electrode and a current through conductor supported with said electrode supporting member.

21. A luminous container comprising a tube-shaped outer supporting body comprising a luminous vessel made of a brittle material, a pipe-shaped inner supporting body provided inside of said outer supporting body and made of a brittle material, and a pipe-shaped metal piece provided between said outer and inner supporting bodies,

wherein the entire outer supporting body is positioned radially outwardly with respect to the inner supporting body, said outer supporting body and said metal piece directly contact each other, said metal piece and said inner supporting body directly contact each other and said outer supporting body and said inner supporting body directly contact each other throughout an entire circumference of the inner supporting body, and

wherein said metal piece functions as an electrode supporting member.

22. The luminous container of claim 21, wherein the difference of thermal expansion coefficients of said outer and inner supporting bodies is 2 ppm/K or lower.

23. The luminous container of claim 21, wherein said plate-shaped metal piece comprises a non-clamped portion comprising a seamless cover portion, wherein a through hole is provided in said cover portion for inserting a current through conductor and an electrode.

24. The luminous container of claim 21, wherein said non-clamped portion comprises a guide for adjusting the concentricity of a current through conductor and an electrode and a capillary portion having a length capable of being a connecting end.

25. An assembly for a luminous container, comprising said luminous container of claim 21, wherein said electrode supporting members are fixed onto one and the other ends of said luminous container, respectively, a current through conductor is inserted into said electrode supporting member in advance, said electrode is contained in said luminous container in advance, and said electrode supporting member and said current through conductor are not sealed in air tight manner in at least one of said one and the other ends.

26. A luminous container for a high pressure discharge lamp, comprising said luminous container of claim 21, and an

30

electrode and a current through conductor supported with said electrode supporting member.

27. A luminous container comprising a tube-shaped inner supporting body comprising a luminous vessel made of a brittle material, a pipe-shaped outer supporting body provided outside of said inner supporting body and made of a brittle material, and a pipe-shaped metal piece provided between said inner and outer supporting bodies,

wherein the entire outer supporting body is positioned radially outwardly with respect to the inner supporting body, said inner supporting body and said metal piece directly contact each other, said metal piece and said outer supporting body directly contact each other and said outer supporting body and said inner supporting body directly contact each other throughout an entire circumference of the inner supporting body, and wherein said metal piece functions as an electrode supporting member.

28. The luminous container of claim 27, wherein the difference of thermal expansion coefficients of said outer and inner supporting bodies is 2 ppm/K or lower.

29. The luminous container of claim 27, wherein said plate-shaped metal piece comprises a non-clamped portion comprising a seamless cover portion, wherein a through hole is provided in said cover portion for inserting a current through conductor and an electrode.

30. The luminous container of claim 29, wherein said non-clamped portion comprises a guide for adjusting the concentricity of a current through conductor and an electrode and a capillary portion having a length capable of being a connecting end.

31. An assembly for a luminous container, comprising said luminous container of claim 27, wherein said electrode supporting members are fixed onto one and the other ends of said luminous container, respectively, a current through conductor is inserted into said electrode supporting member in advance, said electrode is contained in said luminous container in advance, and said electrode supporting member and said current through conductor are not sealed in air tight manner in at least one of said one and the other ends.

32. A luminous container for a high pressure discharge lamp, comprising said luminous container of claim 27, and an electrode and a current through conductor supported with said electrode supporting member.

\* \* \* \* \*